

April 29, 1941.

O. SCHINCKE

**2,240,099**

## METHOD OF BRIGHT ANNEALING ELONGATED METAL BODIES

Filed Sept. 14, 1936

2 Sheets-Sheet 1



INVENTOR

Otto Schuncke,  
By, Watson, Croit, Morse & Gindles.  
ATTYS.

April 29, 1941.

O. SCHINCKE

2,240,099

## METHOD OF BRIGHT ANNEALING ELONGATED METAL BODIES

Filed Sept. 14, 1936

2 Sheets-Sheet 2

Fig. 4a



Fig. 4b



INVENTOR

Otto Schinckel,  
By Patent, Coit, Moore & Ginder.  
ATTYS.

## UNITED STATES PATENT OFFICE

2,240,099

METHOD OF BRIGHT ANNEALING  
ELONGATED METAL BODIES

Otto Schincke, Vienna, Austria

Application September 14, 1936, Serial No. 100,749  
In Austria October 18, 1935

4 Claims. (Cl. 148—16)

This invention relates to the annealing of elongated metal bodies, and more particularly rigid metal bodies such as tubes or rods, with the retention of a bright surface, in the case of hollow bodies of a bright surface both inside and outside.

The method according to the invention is primarily suited for the bright annealing of metal goods made from copper and copper alloys, but also for the treatment of metal bodies made from other metals and alloys such as for example steel.

The invention has for its object to simplify the technique of and to cheapen the annealing process, in which oxidation of the metallic material handled must be inhibited, and makes it possible, first and foremost, for rigid metal bodies of any desired length to be subjected to bright annealing in an uninterrupted working operation without any special precautions having to be taken.

A large number of proposals have already become known for the bright annealing of metallic material. According to a widely practised method of working the annealing is carried out in annealing chambers or pots from which, with the view of avoiding oxidation of the metal treated, the air has been removed either by displacement by a protective gas or by evacuation. The evacuation is generally effected by the connection of an exhausting air pump to the annealing container. In addition, there is also to be found in the existing literature on the subject the proposal to produce the desired reduced pressure in annealing pots by mere heating, the admission of air into the vessel being prevented, after the attainment of the maximum temperature, by closing the outlet valve. With all known methods of this nature the annealing is effected in a chamber which is gas-tightly closed off from the outside atmosphere. Since the dimensions of the chamber or of the receiving container set a limit to the dimensions of the material to be treated only metal bodies of restricted length can be subjected to the annealing treatment by these known working methods. Moreover, when annealing containers are used the annealing process can only be carried out intermittently (in batches).

Annealing furnaces have already been built which admit of continuous operation. For this purpose the procedure adopted has been based on the assumption that, to avoid oxidation of the annealed material, it is not merely necessary to carry out the annealing process in a protective gas atmosphere, but also to take special precau-

tions to prevent the admission of air to the annealing chamber.

Thus for example a furnace design has been recommended in which the two ends of the annealing retort take the form of downwardly bent tubes which extend, with the inlet and outlet orifices for the metal material, under the surface of a liquid bath; by the liquid seal thus provided at both ends of the retort the admission of air to the annealing zone is prevented, while a protective gas is introduced into this zone. A bright annealing furnace of this nature is indeed suited for annealing flexible material such as wire, strip, and the like, but the treatment of elongated rigid bodies is not possible in a furnace of this description.

According to another known type of furnace design the retort is sealed by means of stuffing-boxes the internal clearance of which corresponds to the cross-section of the material to be treated, so that during the passage of the material through the inlet and outlet apertures no air can enter the annealing zone, while at the same time steam or the like is introduced under pressure into the annealing zone through a suitable inlet. When elongated rigid metal bodies are treated in this furnace the individual bars or tubes to be consecutively treated are successively interconnected at the ends, in order to ensure that the orifices of the annealing retort are not disclosed at the transition from one to the other of the individual pieces of material during the continuous working process. When handling tubes, this is effected with the aid of special connecting pieces which are drilled for the admission of water which becomes converted in the annealing zone into steam which acts as a protective gas.

Only for the annealing of fine wire has a proposal become known by which the work is carried on uninterruptedly without the introduction of a protective gas into the annealing chamber; also in this case the wire is introduced and withdrawn through a nozzle the bore of which is adapted to fit exactly the cross-section of the wire, so as to prevent the admission of air, and in addition dusting with talc is done to aid in the formation of a seal against the access of air.

In consequence of the difficulties attendant on all these methods of working, which difficulties are principally concerned with the sealing of the annealing zone from the access of air and become harder to deal with the larger the cross-section of the material to be treated is; it is still in the main the usual practice, even to-day, to

anneal metal tubes or rods of great length in the air and then to remove the oxide skin thereby formed by the difficult and troublesome process of pickling.

The present invention is based upon the surprising discovery that it is possible (contrary to the hitherto accepted opinion) in connection with the bright annealing of metal material within a tubular conduit (for example a retort) to dispense with special precautions for preventing the access of air from the outside atmosphere, for instance by tightly closing the entry and outlet apertures (whether by fluid seals and the like or by means of stuffing-boxes and the like) under certain conditions, namely provided the dimensions of the annealing tunnel, as regards length and inside clearance, be so determined in dependence upon each other that within the heated part there becomes formed a permanently maintained zone of atmosphere of reduced density, as in this case in spite of communication with the outside atmosphere air from the latter does not enter the annealing zone.

The method according to the present invention for the bright annealing of elongated and more particularly rigid metal bodies such as tubes, in which the metal material travels, preferably continuously, through an annealing zone within a tubular tunnel, thus consists essentially in passing the material through a tunnel which is bathed by combustion gases at the annealing zone, and the length and inside clearance of which are so dimensioned in dependence upon each other that in the heated part a permanently maintained zone of atmosphere of reduced density is formed, with the maintenance of an open communication between the tunnel and the outside atmosphere at the entry end or at the entry and discharge ends, whereby an additional introduction of protective gas can be dispensed with.

The retention of a bright surface on the metal, with this method, in the absence of protective gas is apparently ensured by the fact that the oxygen content of the atmosphere in the annealing zone is reduced to such an extent, by the rarefaction of the air due to the heating, which is constantly maintained, that practically speaking oxidation cannot occur. It may also be that neutral or reducing gases, such as hydrogen, contained in the combustion gases penetrate through the tunnel wall into the annealing zone, and aid in the action of the atmospheric rarefaction in the annealing zone, or themselves exert a reducing action. If desired, the air may be displaced at the commencement of the annealing process, in a manner known per se, by the introduction of a protective gas.

It will be clear that it is necessary, in connection with this method, to avoid the setting up of a chimney action (draught) in the annealing zone, which would bring about the feeding in of air. Thus when the annealing tunnel is inclined to the horizontal it is necessary to seal the lower end of the tunnel, in a manner known per se, by means of a liquid. Even with this form of construction of the annealing plant, however, the entry end of the tunnel remains in open communication with the outside atmosphere; likewise with this form of construction an additional introduction of protective gas into the annealing zone is not necessary.

For the annealing of tubes of an outside diameter of say 25 mm. there may be employed for example a tunnel the inside diameter of

which is about 50 mm. and the length of which amounts to some 6 to 10 m., the annealing zone proper attaining a length of about 1 to 2 m., while the remainder of the length of the tunnel 5 is mainly utilized for the cooling of the treated material. If the tunnel is inclined, and sealed at the outlet or discharge end by means of a liquid in which the annealed material is cooled very considerably shorter tunnels of a total length of say 3 to 4 m. will suffice; in this case greater freedom is given for the selection of the ratio between the inside clearance and the length of the tunnel.

Given constant furnace temperature, the annealing temperature assumed by the metallic material in the annealing zone may be adjusted in a manner known per se, by regulating the rate of movement of the metal material through the tunnel, according to the nature of the metal 10 or metal alloy and the dimensions of the material to be treated. For example, a pure copper pipe of an internal diameter of approximately 18 mm. and an external diameter of approximately 20 mm., when the temperature of the furnace is about 900° C., may be conducted through the annealing zone at the rate of about 1 m. a minute, the annealing temperature of the tube material being only about 650° C. If it is desired to anneal at lower temperatures the rate 15 of conveying is suitably increased, and in the converse case the rate of conveying is reduced so that the material assumes a higher temperature which may be increased in this way up to a maximum temperature which is but slightly lower than the furnace temperature. If it is desired to increase the rate of movement through the annealing zone at a given annealing temperature this zone is made correspondingly longer.

The present invention provides the possibility of subjecting metal bodies of any length, for example of a length amounting to 20 m. and more, to the annealing process without interruption, with the retention of a bright surface, and without the necessity of connecting together the individual pieces or lengths of the material or of sealing the entry aperture of the annealing tunnel. The further advantage therefore accrues that a plurality of individual pieces placed side by side can also be annealed simultaneously, provided there is room for them in the annealing tunnel.

Apparatus for carrying out the method according to the invention consists for example of a furnace which is traversed from side to side by a tube made from known heat-resistant materials, and more particularly from heat-resistant steel. To this tube, which comprises the annealing zone proper, further tubes may be permanently or detachably connected at one side or at both sides. Since the extension tubes are not exposed to the direct action of the furnace heat they may also be made from other materials than refractory or heat-resistant material. The tunnel may equally well be formed of a single tube comprising the annealing zone as well as the cooling zone. The tunnel is preferably of circular cross-section, but it is also possible to arrange for it to be of any other cross-sectional configuration.

The heating of the tunnel from the outside is preferably effected by means of gas or crude oil burners, although it is equally possible to fire the furnace with solid fuels such as coal, coke, or the like.

After the furnace has been heated up to the required temperature, having regard for the difference between the temperature in the furnace and that in the annealing zone of the tunnel, whereby the appropriate reduction in the density of the atmosphere in the annealing zone is achieved, the metal material to be subjected to the annealing process is fed continuously into the tunnel, travels through the annealing zone, and passes out continuously at the other end of the tunnel into the cooling means. The cooling may be effected in any known manner, for example by extending the discharge end of the tunnel and surrounding this extension for a suitable distance with a cooling jacket through which a cooling liquid is caused to flow.

It is also advisable to discharge the annealed material from the tunnel directly into a cooling bath which may consist for example of water or oil. The plant is preferably so designed that the discharge end of the tunnel extends just beneath the surface of the cooling bath, so that the annealed material passes directly into this bath. In this case, when water is used as the cooling medium, decomposition of the water vaporized by contact with the hot metal yields hydrogen which exerts a reducing action upon any oxide present.

Other and further objects and features of the invention will be more apparent to those skilled in the art upon consideration of the accompanying drawings and following specification wherein I disclose two exemplary embodiments of an apparatus for carrying out the method according to this invention, with the understanding, however, that such change may be made in the structure as will fall within the scope of the appended claims without departing from the spirit of the invention.

Fig. 1 is a side view of a form of construction of apparatus, partly in vertical section, according to which the annealing tunnel is disposed horizontally; Fig. 2 a section through the furnace on the line 2—2, Fig. 1; Fig. 3 a vertical section through the coupling between the annealing tunnel and the cooling tubes; Fig. 4a a side view of another form of construction of apparatus, partly in vertical section, according to which the axis of the annealing tunnel is inclined to the horizontal, and Fig. 4b a continuation of Fig. 4a showing the portion of the container with the cooling liquid, which is broken off in Fig. 4a, the dotted lines illustrating the broken off end of Fig. 4a.

Referring to Figs. 1 to 3 of the drawings, 10 denotes the furnace which is built up of brick-work 11 and heat insulating material 12, and is encased partly by a shell 13 of sheet metal. The furnace is heated for instance by means of gas or crude oil burners not shown, the flames being injected into the furnace through the nozzles 14. The furnace is traversed by parallel tubes 15 of heat-resistant steel which pass through the end walls of the furnace and constitute the annealing zone within the furnace. Inside the furnace the tubes 15 are supported by the plate 16, and outside the furnace uprights 17 fixed to the end walls of the furnace serve this purpose. The combustion gases bathe the tubes 15 and leave the furnace through the aperture 18. 19 denotes a hole in the furnace wall for the insertion of a pyrometer, and 20 is an observation hole.

The feeding of the elongated rigid metal bodies to be annealed, for instance metal tubes 21, is effected by means of a conveying device consisting of two pairs of co-acting rollers 22, 23 the lower rollers 22 of which are driven through the gear 75

24 and the friction wheels 25 by the driving shaft 26. The friction gearing 25 enables the control of the speed of the rollers 22. The upper rollers 23 are mounted adjustably in height so that the distance between the surfaces of the upper and lower rollers may be regulated according to the thickness of the metal bodies to be treated.

The annealing tubes 15 are connected by the coupling 27 to the tubes 28 which are encased by a cooling jacket 29. Water is supplied to the cooling jacket 29 through the feed pipe 30 and withdrawn through the discharge pipe 31.

As particularly shown in Fig. 3, the coupling 27 consists of two pipe flanges 32 fixed together by the screws 33 which co-act with two sockets 34 each of which being screwed on the end of the annealing tube 15 and the cooling tube 28 respectively. Between the sockets there is inserted a packing member 35.

The free ends 15<sup>a</sup>, 28<sup>a</sup> of the annealing tubes and cooling tubes respectively are open and thus in direct communication with the outside atmosphere.

The form of construction shown in Figs. 4a and 4b is similar to that of Figs. 1 to 3. However, the axes of the annealing tubes 15 and of the cooling tubes 28 are inclined to the horizontal, the inclination being about 8:100, and as cooling means there is used a cooling bath provided in the container 36. Furthermore, the annealing tubes 15 are integral with the cooling tubes 28 so that each tube comprises both the annealing and cooling zones. These tubes are open at the entry end 15<sup>a</sup> as in the above described form of construction, and terminate at the discharge end 28<sup>a</sup> below the surface of the cooling liquid in the container 36. With this form of apparatus the annealed metal tubes 21 or the like pass directly into the cooling bath, travel through the same and are conveyed out of it along the bottom of the container 36 which is slightly concave for this purpose. At the end of the bottom of the container is even again so that the metal tubes 21 leave the cooling bath in straight condition.

What I claim is:

1. A method of bright annealing elongated rigid metal bodies comprising heating externally by combustion gases a long, straight and horizontal annealing tunnel of heat-resisting steel, to a temperature at which the density of the atmosphere is reduced to a degree at which a non-oxidizing condition is reached in the tunnel, maintaining said condition, cooling a straight tunnel tightly connected to and in alignment with said annealing tunnel, maintaining an open communication with the outside atmosphere at the entry end of the annealing tunnel and the discharge end of the cooling tunnel, introducing the said elongated metal bodies into the annealing tunnel through the entry end thereof, moving said metal bodies through said annealing and cooling tunnels at a rate controlled so that said metal bodies assume the proper annealing temperature, and discharging the metal bodies through the outlet end of said cooling tunnel.

2. A method of bright annealing elongated rigid metal bodies comprising heating a long straight annealing tunnel, tightly connected to and in alignment with a straight cooling tunnel, externally by combustion gases to a temperature at which the density of the atmosphere is reduced to such a degree that a non-oxidizing condition is reached in the tunnel, providing an open communication with the outside atmosphere at

least at the entry end of the annealing tunnel, maintaining a non-oxidizing condition in the tunnel by the continued application of heat thereto and by the prevention of a longitudinal draft therethrough, introducing the said elongated metal bodies into the annealing tunnel through the entry end thereof, moving said metal bodies through said straight annealing and cooling tunnels at a rate controlled so that said metal bodies become heated to the proper annealing temperature in the annealing tunnel, and discharging the metal bodies through the outlet end of said cooling tunnel.

3. A method of bright annealing elongated rigid metal bodies comprising heating a long straight annealing tunnel, tightly connected to and in alignment with a straight cooling tunnel, externally by combustion gases to a temperature at which the density of the atmosphere is reduced to such a degree that a non-oxidizing condition is reached in the tunnel, providing an open communicating with the outside atmosphere at least at the entry end of the annealing tunnel, maintaining a non-oxidizing condition in the heated portion of the tunnel by the continued application of heat thereto and, by disposing the entry and outlet ends of the tunnel at the same elevation or sealing with liquid the outlet opening if lower than the entry opening, preventing the formation of a draft longitudinally of the tunnel, introducing the said elongated metal bodies into the annealing tunnel through the entry end thereof, moving said metal bodies through said straight annealing and cooling tunnels at a rate controlled so that said

metal bodies become heated to the proper annealing temperature in the annealing tunnel, and discharging the metal bodies through the outlet end of said cooling tunnel.

4. The method of bright annealing elongated rigid metal bodies the surfaces of which will oxidize if brought into contact with air under atmospheric conditions while heated to annealing temperature, which comprises heating externally by hydrogen-containing combustion gases a portion of a straight tunnel or muffle made of heat-resisting steel, the interior of the said tunnel or muffle being at all times in free communication with the outside atmosphere at least as to the heated portion thereof, raising the temperature within said tunnel to a minimum temperature of 900° C. to render the air therein non-oxidizing, maintaining a non-oxidizing condition in the heated portion of the tunnel by the continued application of heat thereto and, by disposing the entry and outlet ends of the tunnel at the same elevation or sealing with liquid the outlet opening if lower than the entry opening, preventing the formation of a draft longitudinally of the tunnel, maintaining cooling temperatures in the unheated portion thereof, and passing an article to be bright annealed through the tunnel or muffle, the direction and rate of movement being such that the article is first raised to annealing temperatures in the rarefied atmosphere of the heated portion and thereafter allowed to cool in the unheated portion before being discharged into the outside atmosphere.

OTTO SCHINCKE.